

## UNITED STATES PATENT OFFICE

2,688,541

## LIGHT-SENSITIVE COLOR PHOTOGRAPHIC MATERIAL

Karl Otto Gauguin and Eric Macdonald, Blackley, Manchester, England, assignors to Imperial Chemical Industries Limited, a corporation of Great Britain

No Drawing. Application November 13, 1951,  
Serial No. 256,127

Claims priority, application Great Britain  
November 20, 1950

5 Claims. (Cl. 95—2)

1

This invention relates to colour photography and more particularly to a simplified multilayer material for use in colour photography.

In multilayer photographic films or paper adapted for use in colour photography which comprise differently sensitised emulsion layers mounted on a film base or paper and wherein the uppermost layer is used for forming the blue record, a yellow filter layer is usually employed between the uppermost (blue sensitive) layer and the other sensitive layers, which in addition to being sensitised to other parts of the spectrum are also sensitive to blue light. The yellow filter layer absorbs the blue light and prevents it striking these lower sensitive layers.

The coating of the yellow filter layer itself provides an undesirable complication of the process of manufacture of the photographic film or paper and when colloidal silver is used in the yellow filter layer, as is usual in commercial processes, further complications are introduced by the necessity of coating separation layers between the filter layer and the light sensitive layers to avoid fogging of the sensitive emulsions by the colloidal silver.

It is known that when a yellow dyestuff, even in high concentration, is introduced into a single light-sensitive gelatino-silver halide emulsion layer, the layer is still partially sensitive to the blue light striking the light sensitive silver halide at or near the surface of the layer, but we have found that when a blue sensitive layer is coated on top of a light sensitive layer containing a yellow styryl dyestuff as hereinafter defined, the latter layer is entirely or almost unaffected by normal exposure to blue light which has passed through the superimposed blue sensitive layer. By a blue sensitive layer we mean a layer of light sensitive gelatino-silver halide emulsion which has not been spectrally sensitised to parts of the spectrum other than blue.

According to our invention we provide a photographic material adapted for use in colour photography which comprises three differently sensitised gelatino-silver halide emulsion layers containing yellow, magenta and cyan colour formers superimposed on a support, characterised in that one of the outermost sensitive layers is sensitive to blue light and is adjacent to, and not separated by a filter layer from the middle sensitive layer which middle sensitive layer contains a yellow styryl dyestuff as hereinafter defined.

The yellow styryl dyestuffs used in the process of the present invention which function both as a yellow filter dyestuff and as a magenta colour former are the water soluble dyestuffs which carry

2

a substituent rendering the dyestuff non-diffusible, for example a substituent containing an alkyl chain of at least 5 carbon atoms, and which are obtainable by condensing a reactive methylene compound with an anil of a water-soluble or alkali-soluble aldehyde of the formula



10 wherein the benzene nucleus may be substituted and wherein at least one of the radicals R<sub>1</sub> and R<sub>2</sub> is an alkyl radical substituted with for example, —CN, —COOAlkyl, —NO<sub>2</sub> carboxyl or sulphonate acid groups, and, when only one of the radicals R<sub>1</sub> and R<sub>2</sub> is an alkyl radical so substituted, the other radical is a substituted or unsubstituted hydrocarbon radical.

15 Suitable styryl dyestuffs may be obtained by condensing an anil of a p-substituted-amino-benzaldehyde with a reactive methylene compound of the kind used for forming magenta dyestuffs in colour photography by reaction with colour developers. These reactive methylene compounds may be for example, compounds of the pyrazolone series or of the cyanoacetyl-series.

20 Specific examples of suitable reactive methylene compounds are 1-(4'-phenoxy-3'-sulphophenyl)-3-heptadecyl-5-pyrazolone, 1-(phenyl-3'-methanesulphonic acid)-3-heptadecyl-5-pyrazolone, and the compound obtained by acylating 4-omega-cyanoacetaniline with octadecenylsuccinic anhydride.

25 As suitable p-substituted-amino-benzaldehydes there may be mentioned for example p-(N-methyl-N-sulphoethyl-amino)-benzaldehyde, p-(N:N-β:β'-disulphodiethylamino)-benzaldehyde, 4-(N:N'-β:β'-disulphodiethylamino)-2-methyl-benzaldehyde, p-(N-methyl-N-carboxyethylamino)-benzaldehyde, p-(N:N-β:β'-dicarboxydiethylamino)-benzaldehyde, p-N:N-di(carboxymethyl)-amino-benzaldehyde, p-(N-β-sulphoethylamino)-benzaldehyde, 4-(N:N-β:β'-dichlorodiethylamino)-2-sulpho-benzaldehyde.

30 35 40 45 50 55 p-N:N-di-(carboxymethyl)-amino-benzaldehyde may be made by introducing the aldehyde group into di-(ethylcarboxymethyl)-aniline by the method of Vilsmeier and Haack (Berichte, volume 60, page 119) and hydrolysing the diester so obtained. The other mono- or di-(carboxy-alkyl) derivatives may be made by hydrolysis of the appropriate cyanoalkyl compounds which may be made by treating the corresponding hydroxyalkyl or dihydroxydialkyl anilines with phosphorus pentabromide, treating the corresponding bromoalkyl or dibromodialkyl com-

pounds so obtained with potassium cyanide, and introducing the aldehyde group by reaction with phosphorus oxychloride and N-methylformanilide and subsequent hydrolysis, that is to say by the methods of Vilsmeier and Haack (Berichte, volume 60, page 119). The mono- and di-(sulphoalkyl) derivatives may be made by the action of sodium sulphite on the corresponding chloroalkyl compounds.

It will be apparent that if the top layer is 10 blue sensitive, the material will be exposed in the normal way to light, but if the bottom layer is blue sensitive, the material will be exposed to light through the support.

In one embodiment of our invention in which the photographic material is especially valuable for use in the production of colour positive transparencies and prints, there are 3 sensitive layers superimposed on the support, the top layer being blue sensitive (that is not spectrally sensitised) and containing a yellow colour former, the middle layer containing a styryl dyestuff as hereinbefore defined, which serves both as a yellow filter dyestuff and as a magenta colour former and the bottom layer containing a cyan colour former, either the middle layer or the bottom layer being red sensitive and the other being green sensitive.

Such a photographic material may be exposed and processed by known means when the filter dyestuff is largely discharged in the developing process. To ensure complete discharge of the dyestuff the material, may, if desired, be treated after the development step with hydrazine hydrate which may if desired be added to the fixing bath.

If the spectral absorption of the magenta dyestuff obtained from the yellow styryl dyestuff is not entirely suitable for a positive print or transparency, then some modification is possible by the addition to the yellow styryl dyestuff of a small proportion of a colourless colour former yielding a suitable magenta dyestuff.

In a second embodiment of our invention, in which the photographic material is especially valuable for the production of negative transparencies, there are 3 sensitive layers superimposed on a support, the top layer being blue sensitive (that is not spectrally sensitised) and containing a yellow colour former, the middle layer containing a mixture of a yellow styryl dyestuff as hereinbefore defined and a yellow styryl dyestuff derived from a reactive methylene compound and a water-insoluble and alkali-insoluble p-N-substituted amino-benzaldehyde, and the bottom layer containing a cyan colour former, either the middle layer or the bottom layer being red sensitive and the other being green sensitive.

Examples of suitable water-insoluble and alkali-insoluble p-N-substituted amino-benzaldehyde are p-(N-methyl-N-β-hydroxyethylamino)-benzaldehyde, p-(N-ethyl-N-β-hydroxyethylamino)-benzaldehyde, p-(β:β'-dihydroxydiethylamino)-benzaldehyde, p-(N-methyl-N-methoxyethylamino)-benzaldehyde, p-(N-ethyl-N-methoxyethylamino)-benzaldehyde, p-(N-butyl-N-β-hydroxyethylamino)-benzaldehyde, p-(N-methyl-N-β-chloroethylamino)-benzaldehyde, p-(N-ethyl-N-β-chloroethylamino)-benzaldehyde, p-(β:β'-dichlorodiethylamino)-benzaldehyde, 4-(β:β'-dichlorodiethylamino)-2-methylbenzaldehyde, p-(N-methyl-N-β-cyanoethylamino)-benzaldehyde, p-(β:β'-dicyanodiethylamino)-benzaldehyde and p-di-(ethylcarboxymethyl)-amino-benzaldehyde.

Such a photographic material may be exposed

and developed, bleached and fixed by known means and then treated with formaldehyde or sodium nitrite when a yellow colour correction mask is formed in the middle layer. It is suggested as a possible explanation of this process that both styryl dyestuffs function as filter dyestuffs and colour formers and that in the development with an aromatic amine as developer, magenta images are formed in the exposed parts of the middle layer by the action of the oxidation product of the developer on the styryl dyestuffs and the rest of the styryl dyestuffs are decomposed by the developer to give the parent reactive methylene compounds and also anils formed from the parent aldehydes by reaction with the developer. The anil from the soluble aldehyde is washed out from the photographic material during the processing steps. The insoluble aldehyde is liberated from the corresponding anil by the action of formaldehyde or sodium nitrite and it then reacts with the reactive methylene compound to re-form the yellow styryl dyestuff. Since the concentration of residual reactive methylene compound will be much higher in the counter-imagewise parts of the layer than in the imagewise parts (where it has been used for forming magenta dyestuffs) then the intensity of yellow styryl dyestuff formed will be higher in the counter-imagewise parts and accordingly the styryl dyestuff will form a colour correction masking image.

It will be apparent that the strength of the masking image can be controlled by adjusting the proportions of the two styryl dyestuffs in the 35 layer.

The invention is illustrated but not limited by the following examples in which the parts are by weight:

#### Example 1

40 A multilayer light sensitive photographic paper is made up as follows:

A red sensitive gelatino-silver halide emulsion layer containing 10 grams per litre of the sodium 45 salt of the cyan colour forming component 1-hydroxy-4-sulpho-2-naphthyoctadecylamide is coated on a paper support and on this layer there is coated a gelatin separation layer and subsequently a green sensitive gelatino-silver halide emulsion layer containing 15 grams per litre of the sodium salt of the yellow styryl dyestuff 1-(4'-phenoxy-3'-sulphophenyl)-3-heptadecyl-4-p-N:N'-di-(carboxyethyl)-amino-benzylidene-5-pyrazolone, to act both as the 50 magenta colour forming component and also as the yellow filter dyestuff. A gelatin separation layer is then coated and finally as the top layer there is coated a blue sensitive gelatino-silver halide emulsion containing 10 grams per litre of p-stearylamino-benzoylacetanilide-p'-carboxylic acid sodium salt, the yellow colour forming component described in Example 3 of British specification No. 486,848.

60 The paper is exposed to the light transmitted by a subtractively coloured negative transparency and then developed in a solution of the following composition:

|                                             | Parts |
|---------------------------------------------|-------|
| p - N:N - diethylaminoaniline hydrochloride | 3     |
| Sodium sulphite, anhydrous                  | 2     |
| Hydroxylamine hydrochloride                 | 1     |
| Sodium carbonate, anhydrous                 | 60    |
| Potassium bromide                           | 0.5   |
| Water to make up to                         | 1000  |

## 5

The paper is rinsed and transferred to a stop bath of the following composition:

|                      | Parts |
|----------------------|-------|
| Acetic acid, glacial | 15    |
| Sodium acetate       | 30    |
| Water to make up to  | 1000  |

The paper is washed and transferred to a bleaching solution of the following composition:

|                             | Parts |
|-----------------------------|-------|
| Potassium ferricyanide      | 100   |
| Potassium bromide           | 25    |
| Sodium dihydrogen phosphate | 50    |
| Water to make up to         | 1000  |

The paper is further washed and treated in a fixing and dyestuff discharge solution of the following composition:

|                                | Parts |
|--------------------------------|-------|
| Sodium thiosulphate            | 200   |
| 50% hydrazine hydrate solution | 100   |
| Water to make up to            | 1000  |

The paper is finally washed and dried when a positive paper print is obtained.

## Example 2

A multilayer light sensitive photographic material is made up as follows:

A red sensitive gelatino-silver halide emulsion layer containing 10 grams per litre of the sodium salt of the cyan colour forming component obtained by condensing 1-hydroxy-2-naphthoic acid chloride with oleylamine and sulphonating (that is the colour forming component described in Example 10 of British specification No. 465,823), is coated on a transparent support and on this layer there is coated a green sensitive gelatino-silver halide emulsion layer containing 12 grams per litre of the styryl dyestuff 1-(4'-phenoxy - 3' - sulphophenyl) - 3 - heptadecyl - 4 - p - di(β - cyanoethyl) - amino - benzylidene-5-pyrazolone sodium salt, derived from the insoluble aldehyde p-di-(β-cyanoethyl)-amino-benzaldehyde and 5 grams per litre of the styryl dyestuff 1-(4'-phenoxy-3'-sulphophenyl)-3-heptadecyl - 4 - p - di - (carboxyethyl) - amino - benzylidene-5-pyrazolone sodium salt, derived from the soluble aldehyde p-(β:β'-dicarboxydiethyl-amino)-benzaldehyde. This layer serves as a yellow filter layer, and provides the magenta colour forming components and also the yellow masking dyestuff. Finally as the top layer there is coated a blue sensitive gelatino-silver halide emulsion containing 10 grams per litre of p-stearylamino-benzoylacetanilide-p-carboxylic acid sodium salt (the yellow colour forming component described in Example 3 of British specification No. 486,848). The film is exposed to the light from a coloured object and developed in a developer solution of the following composition:

|                                          | Parts |
|------------------------------------------|-------|
| p-N:N-diethylaminocaniline hydrochloride | 3     |
| Sodium sulphite, anhydrous               | 1     |
| Sodium carbonate, anhydrous              | 60    |
| Potassium bromide                        | 2     |
| Water to make up to                      | 1000  |

The film is washed, bleached in a bleaching solution of the composition used in Example 1, washed, fixed with sodium thiosulphate and then treated with a 1% solution nitrite. This treatment with sodium nitrite regenerates the styryl dyestuff derived from the insoluble aldehyde but not that from the soluble aldehyde, since the anil formed from the soluble aldehyde and the amine

## 6

of the developer solution has been removed during the processing and washing steps.

The processed material contains in the first layer a cyan dyestuff negative image, in the second layer a magenta dyestuff negative image and a yellow styryl dyestuff positive image and in the top layer a yellow dyestuff negative image.

## Example 3

A multilayer material is made up as described in Example 1, but in place of the yellow styryl dyestuff described there is used 15 grams per litre of the dyestuff 1-β-octadecenyl-succinamide-4-omega-cyano-omega-(p-N:N-di-(carboxyethyl)-amino-benzylidene)-acetobenzene(sodium salt). The paper is exposed to the light transmitted by a subtractively coloured negative transparency and then developed in a solution of the following composition:

|                                             | Parts |
|---------------------------------------------|-------|
| 5-diethylamino-2-aminotoluene hydrochloride | 2.5   |
| Sodium sulphite, anhydrous                  | 2     |
| Hydroxylamine hydrochloride                 | 1     |
| Sodium carbonate, anhydrous                 | 60    |
| Potassium bromide                           | 2     |
| Water to make up to                         | 1000  |

The paper is rinsed and transferred to a stop bath of the following composition:

|                             | Parts |
|-----------------------------|-------|
| Potassium ferricyanide      | 100   |
| Potassium bromide           | 25    |
| Sodium dihydrogen phosphate | 50    |
| Water to make up to         | 1000  |

The paper is further washed and treated in a fixing and dyestuff discharge solution of the following composition:

|                                | Parts |
|--------------------------------|-------|
| Sodium thiosulphate            | 200   |
| 50% hydrazine hydrate solution | 100   |
| Water to make up to            | 1000  |

The paper is finally washed and dried, when a positive paper print is obtained.

## Example 4

In addition to the yellow styryl dyestuff of Example 3 there may be added 3 grams of the colourless colour former 1-(4'-phenoxy-3'-sulphophenyl) - 3 - heptadecyl-5-pyrazolone(sodium salt).

What we claim is:

1. A photographic material adapted for use in colour photography which comprises three superimposed differently sensitized gelatino-silver halide emulsion layers, the layers comprising a middle sensitive layer between two outermost sensitive layers, said layers containing colour formers which couple with the oxidation product of a primary aromatic amino developer to form the color image and are adapted to yield, upon exposure and development, yellow, cyan and magenta coloured images in separate layers, said material being characterized in that one of the outermost sensitive layers is sensitive to blue light and is adjacent to, and not separated by a filter layer from, the middle sensitive layer, which middle sensitive layer contains a water-soluble yellow styryl dyestuff carrying a substituent which renders the dyestuff non-diffusible and obtainable by condensing a reactive methylene compound selected from the group consisting of compounds of the pyrazolone and cyanoacetyl series, with an anil of an aldehyde selected from

the group consisting of water-soluble and alkali-soluble aldehydes of the formula:



wherein R is selected from the group consisting of an unsubstituted monocyclic aryl radical and a sulphonic acid substituted monocyclic aryl radical, at least one of the radicals R<sub>1</sub> and R<sub>2</sub> is a substituted alkyl, said substituent being selected from the group consisting of cyano, carboxy alkyl, nitro, chloro, carboxyl and sulphonic acid groups, and when only one of the radicals R<sub>1</sub> and R<sub>2</sub> is said substituted alkyl, the other radical is a hydrocarbon radical wherein one of R, R<sub>1</sub> and R<sub>2</sub> in all cases contains a member from the group consisting of carboxyl and sulphonic acid groups in the case of R<sub>1</sub> and R<sub>2</sub> and a sulphonic acid group in the case of R.

2. A photographic material as defined in claim 1, wherein the top layer is blue sensitive and contains a colour former adapted to yield a yellow coloured image upon exposure and development and the bottom layer contains a colour former adapted to yield a cyan coloured image upon exposure and development, one of the layers other than the top layer being red sensitive and the other layer being green sensitive.

3. A photographic material as described in claim 2, wherein the middle layer contains a colourless colour former in addition to the styryl dyestuff.

4. A photographic material as described in claim 1, wherein the top layer is blue sensitive

5 10 15 20 25

and contains a colour former adapted to yield a yellow coloured image upon exposure and development, the bottom layer contains a colour former adapted to yield a cyan coloured image upon exposure and development, and the middle layer contains a mixture of said yellow styryl dyestuff and a yellow styryl dyestuff which is the condensation product of a reactive methylene compound and a water-insoluble and alkali-insoluble p-N-substituted amino-benzaldehyde, the substituent on the p-N atom being selected from the group consisting of alkyl, chloroalkyl, hydroxyalkyl, alkoxyalkyl, cyanoalkyl, and alkyl carboxyalkyl groups, one of the layers other than the top layer being red sensitive and the other layer being green sensitive.

5. The photographic material as described in claim 4, wherein the condensation product of the reactive methylene compound and the water-insoluble and alkali-insoluble p-N-substituted amino-benzaldehyde contains a substituent which renders the dyestuff non-diffusible.

#### References Cited in the file of this patent

#### UNITED STATES PATENTS

| Number    | Name          | Date           |
|-----------|---------------|----------------|
| 2,036,546 | Schneider     | Apr. 7, 1936   |
| 2,186,781 | Schneider     | Jan. 9, 1940   |
| 2,428,054 | Vittum et al. | Sept. 30, 1947 |
| 2,449,966 | Hanson        | Sept. 21, 1948 |

#### FOREIGN PATENTS

| Number  | Country       | Date          |
|---------|---------------|---------------|
| 513,596 | Great Britain | Oct. 17, 1939 |